# EUROPEAN PATENT SPECIFICATION

(11) **EP 2 307 595 B1**
(45) Date of publication and mention of the grant of the patent: **10.04.2013**
(21) Application number: 09802519.0
(22) Date of filing: 29.07.2009
(51) Int. Cl.: D04H 3/16, D04H 1/54, D04H 13/00, D04H 3/007, D04H 1/541, D04H 1/544, D01F 8/06, D01D 5/30

(54) **BICOMPONENT FIBERS WITH AN EXTERIOR COMPONENT COMPRISING POLYPROPYLENE**
ZWEI-KOMPONENTEN-FASERN MIT EINER POLYPROPYLENHALTIGEN AUSSENKOMPONENTE
FIBRES BICOMPOSANTS DOTÉES D UN COMPOSANT EXTÉRIEUR COMPRENANT DU POLYPROPYLÈNE

(30) Priority: 29.07.2008 EP 08161327
(43) Date of publication of application: 13.04.2011
(73) Proprietor: TOTAL RESEARCH & TECHNOLOGY FELUY, 7181 Seneffe (BE)
(72) Inventor: HAUBRUGE, Hugues, B-1457 Walhain (BE); PAVY, Guillaume, B-1050 Bruxelles (BE)
(74) Representative: Leyder, Francis
(86) International application number: PCT/EP2009/059805
(87) International publication number: WO 2010/012769

(56) References cited:
- WO-A-00/40789
- WO-A-00/63471
- WO-A-99/06617
- WO-A-03/010370
- US-A- 5 281 378

## Description

### Field of the invention

The present invention relates to bicomponent fibers with improved bonding properties. In particular, the present invention relates to bicomponent fibers comprising an exterior component, which in turn comprises a polypropylene that has been degraded from a first melt flow index MFI₁ (measured according to ISO 1133, condition L, 230°C, 2.16 kg) to a second melt flow index MFI₂ (measured according to ISO 1133, condition L, 230°C, 2.16 kg), such that the degradation ratio MFI₁/MFI₂ is within a well-defined range and such that the second melt flow index MFI₂ is in the range from 50 dg/min to 300 dg/min. Further, the present invention relates to nonwovens, composites and laminates comprising said bicomponent fibers. The present invention also relates to a process for making such bicomponent fibers, nonwovens, composites and laminates.

### The technical problem and the prior art

Polypropylene is one of the most widely used synthetic polymers for fibers and nonwovens because it has good mechanical and chemical properties and can be easily processed. Mostly, the production of polypropylene fibers and nonwovens is done by a melt extrusion process, wherein molten polypropylene is extruded through a number of fine capillaries to form fibers or filaments, which can then be collected to form a nonwoven.

Depending upon the final application the polypropylene fibers and nonwovens need to have certain properties. For example fibers and nonwovens used in baby diapers should at the same time be strong, and also have a soft touch and good nonwoven forming properties, such as good thermal bonding behavior.

Frequently, it is not possible to produce fibers or nonwovens having all the desired properties with a single polypropylene and one has to revert to technically more demanding solutions, such as for example bicomponent fibers. Bicomponent fibers and nonwovens are made of an exterior component and an interior component with the interior component being largely covered by the exterior component. Such an arrangement allows producing fibers and nonwovens wherein the interior component provides the mechanical strength, and the exterior component provides the thermal bonding properties and/or the soft touch etc. This is exemplified by bicomponent fibers and nonwovens having a polypropylene as interior component and a polyethylene as exterior component.

However, fibers and nonwovens comprising polyethylene have the disadvantage that they are more difficult to produce because the processability of polyethylene in fiber spinning is not as good as that of polypropylene. In addition, in view of the requirements for recycling of consumer products, it is desired to have fibers and nonwovens that are mono-material, i.e. that are made from polypropylene only.

The industry therefore has a need for bicomponent fibers and nonwovens that are easy to produce and have good properties.

It is therefore an object of the present invention to provide bicomponent fibers and nonwovens that can be easily produced.

It is a further object of the present invention to provide bicomponent fibers and nonwovens that have an exterior component comprising polypropylene, with the exterior component having good thermal bonding properties.

It is also an object of the present invention to provide bicomponent fibers and nonwovens with improved mechanical properties.

### Brief description of the invention

We have now discovered that at least one of the above objectives can be met when the bicomponent fibers and nonwovens comprise an exterior component, which in turn comprises a polypropylene having specific properties.

The present invention therefore provides a bicomponent fiber comprising
(a) an exterior component covering at least 50 % of the surface of the bicomponent fibers, and
(b) an interior component comprising a thermoplastic polymer,
wherein the exterior component comprises a polypropylene, which has been degraded chemically or thermally from a first melt flow index MFI₁ (measured according to ISO 1133, condition L, 230°C, 2.16 kg) to a second melt flow index MFI₂ (measured according to ISO 1133, condition L, 230°C, 2.16 kg), such that the second melt flow index MFI₂ is in the range from 50 dg/min to 300 dg/min and such that the degradation ratio MFI₁/MFI₂ is at least 0.10 and at most 0.80..

The present invention further provides spunbond nonwovens, composites and laminates comprising such bicomponent fibers.

In addition, the present invention provides a process for the production of bicomponent fibers comprising the steps of
(a) polymerizing propylene and one or more optional comonomers with a polymerization catalyst to produce a polypropylene having a first melt flow index MFI₁ (measured according to ISO 1133, condition L, 230°C, 2.16 kg),
(b) thermally or chemically degrading the polypropylene obtained in step (a) to a second melt flow index MFI₂ (measured according to ISO 1133, condition L, 230°C, 2.16 kg),
(c) melting a polypropylene composition comprising the polypropylene obtained in step (b) in a first extruder to form a molten polypropylene composition,
(d) melting a thermoplastic polymer composition comprising a thermoplastic polymer in a second extruder to form a molten thermoplastic polymer composition,
(e) extruding the molten thermoplastic polymer composition from a number of fine, usually circular, capillaries of a spinneret,
(f) extruding the molten polypropylene composition of step (c) from a number of fine openings surrounding said capillaries of step (e), and
(g) combining the extrudates of steps (e) and (f) to form a single filament of an intermediate diameter, such that the extrudates of step (f) form an exterior component covering at least 50 % of the surface of the so-produced filament,
wherein the polypropylene obtained in step (b) has a second melt flow index MFI₂ (measured according to ISO 1133, condition L, 230°C, 2.16 kg) in the range from 50 dg/min to 300 dg/min and wherein the degradation ratio MFI₁/MFI₂ is at least 0.10 and at most 0.80.

Further, the present invention provides a process for the production of nonwovens, composites and laminates comprising the bicomponent fibers of the present invention.

### Detailed description of the invention

For the purposes of the present invention the terms "fiber" and "filament" may be used interchangeably.

The bicomponent fibers of the present invention comprise an exterior component and an interior component. The exterior component covers at least 50 % of the surface of the bicomponent fibers. More preferably it covers at least 70 %, even more preferably at least 90 %, 95 %, 97 % or 99 % and most preferably 100 % of the surface.

Bicomponent fibers are known in many different configurations, such as for example side-by-side, sheath-core, islands-in-the-sea, pie or stripe configurations. Bicomponent fibers can be formed by co-extrusion of two different components into one fiber or filament. This is done by separately feeding the components to two extruders and combining the melts (or extrudates) into a single fiber or filament. The resulting fiber or filament has two different, essentially continuous polymer phases. Such fibers, their production as well as their forming a nonwoven, are well known to the skilled person and are for example described in F. Fourné, Synthetische Fasern, Carl Hanser Verlag, 1995, chapter 5.2 or in B.C. Goswami et al., Textile Yarns, John Wiley & Sons, 1977, p. 371-376.

### EXTERIOR COMPONENT

The exterior component of said bicomponent fiber comprises a polypropylene. This means that the exterior component is a polypropylene composition. Preferably, the exterior component comprises at least 50 wt%, more preferably at least 70 wt% or 90 wt%, even more preferably at least 95 wt% or 97 wt% or 99 wt% of polypropylene relative to the total weight of the exterior component; it is most preferred that the exterior layer consists of polypropylene.

The polypropylene used in the exterior component may be produced by polymerizing propylene and one or more optional comonomers as defined below in the presence of a Ziegler-Natta catalyst system. Such catalyst systems are well known to the person skilled in the art. They comprise a titanium compound having at least one titanium-halogen bond and an internal electron donor, both on a suitable support (for example on a magnesium halide in active form), an organoaluminium compound (such as an aluminium alkyl), and an optional external donor (such as a silane or a diether compound).

The polymerization of propylene and one or more optional comonomers can be carried out in a slurry, bulk or gas phase process. In a slurry process the polymerization is carried out in a diluent, such as an inert hydrocarbon. In a bulk process the polymerization is carried out in liquid propylene as reactor medium.

For the purpose of the present invention the polypropylene recovered from the polymerization reactor is degraded either by thermal or by chemical treatment. Degradation by chemical treatment ("visbreaking") is preferred. For chemical degradation the molten polypropylene is mixed with a peroxide (for example with 2,5-dimethylhexane-2,5-di-tert-butylperoxide), leading to the generation of radicals, which in turn leads to a breakdown of the polypropylene polymer chains. Thus, the melt flow of the polypropylene increases and the molecular weight distribution narrows. Visbreaking of polypropylene is generally carried out at temperatures in the range from 200°C to 250°C. It can for example be done in the extruder in the granulation step of a polypropylene manufacturing plant or in the extruder feeding a fiber or nonwoven production line.

The degree to which a polypropylene has been degraded can be described by the degradation ratio MFI₁/MFI₂, which is the ratio between a first melt flow index MFI₁ (measured according to ISO 1133, condition L, 230°C, 2.16 kg) before degradation and a second melt flow index MFI₂ (measured according to ISO 1133, condition L, 230°C, 2.16 kg) after degradation. The polypropylene used in the exterior component of the present invention has a degradation ratio MFI₁/MFI₂ of at least 0.1, preferably at least 0.12, more preferably at least 0.14, even more preferably of at least 0.16, still even more preferably of at least 0.18, and most preferably at least 0.20. The polypropylenes used in the present invention have a degradation ratio MFI₁/MFI₂ of at most 0.8, more preferably of at most 0.7, even more preferably of at most 0.6, and most preferably of at most 0.5.

The second melt flow index MFI₂ (measured according to ISO 1133, condition L, 230°C, 2.16 kg) of the polypropylenes used in the exterior component is at least 50 dg/min, preferably at least 55 dg/min, and most preferably at least 60 dg/min. The second melt flow index MFI₂ of the polypropylenes used in the present invention is at most 300 dg/min, preferably at most 200 dg/min, more preferably at most 150 dg/min and most preferably at most 100 dg/min.

### INTERIOR COMPONENT

The interior component of said bicomponent fiber comprises a thermoplastic polymer that adheres to polypropylene. This means that the interior component is a thermoplastic polymer composition.

Preferably, said thermoplastic polymer is selected from the group consisting of polypropylene, polyethylene, polyamide, polyester and polycarbonate. More preferably, the thermoplastic polymer is a polypropylene or a polyethylene. More preferably, it is a polypropylene. Most preferably, said thermoplastic polymer is a polypropylene that is different from the polypropylene comprised in the exterior component. Overall, the thermoplastic polymer is preferably chosen in such a way that the composition of the interior and the composition of the exterior component are different from one another.

Descriptions of these thermoplastic polymers can for example be found in Stoeckhert, Kunststoff Lexikon, W. Woebcken (ed.), 9th edition, Carl Hanser Verlag, München, Wien, 1998 or in Römpp Chemie Lexikon, J. Falbe and M. Regitz (eds.), 9th edition, Georg Thieme Verlag, Stuttgart, New York 1995. They are therefore considered to be are well known to the person skilled in the art so that they need not be described in further detail.

Preferably, the interior component comprises at least 50 wt%, more preferably at least 70 wt% or 90 wt%, even more preferably at least 95 wt% or 97 wt% or 99 wt% of said thermoplastic polymer, relative to the total weight of the interior component; it is most preferred that the interior layer consists of said thermoplastic polymer.

The thermoplastic polymer suitable for use in the interior component has a melt flow index (measured according to ISO 1133, condition L, 230°C, 2.16 kg) in the range from 5 dg/min to 500 dg/min. When used for the production of fibers the thermoplastic polymer used in the interior component preferably has a melt flow index in the range from 5 dg/min 40 dg/min. When used in the spunbonding process the thermoplastic polymer used in the interior component preferably has a melt flow index of at least 10 dg/min, more preferably of at least 15 dg/min and most preferably of at least 20 dg/min; preferably the melt flow index is at most 300 dg/min, more preferably at most 200 dg/min, even more preferably at most 100 dg/min and most preferably at most 60 dg/min.

If the thermoplastic polymer is a polypropylene, it preferably has a molecular weight distribution (M_{w}/Mₙ) in the range from 2.0 to 8.0, more preferably in the range from 2.0 to 5.0. Such a polypropylene can for example be produced with a metallocene catalyst or with a Ziegler-Natta catalyst. When produced with a Ziegler-Natta catalyst it is preferred that the molecular weight distribution is reduced by thermal or chemical post-reactor treatment, for example by degradation with a peroxide ("visbreaking"). Molecular weights may be determined by size exclusion chromatography (SEC) as described in the examples.

The polypropylenes used in the present invention, irrespectively of whether used in the exterior or the interior component, can either be homopolymers or random copolymers of propylene with one or more comonomers. Homopolymers are preferred.

The comonomers can be ethylene or a C₄ - C₂₀ α-olefin, such as for example butene-1, pentene-1, hexene-1, octene-1 or 4-methyl-pentene-1. The preferred random copolymer is a copolymer of propylene and ethylene. The random copolymers of the present invention comprise at least 0.1 wt%, preferably at least 0.2 wt% and most preferably at least 0.5 wt% of comonomer. Preferably they comprise at most 6.0 wt%, more preferably at most 5.0 wt% and most preferably at most 4.0 wt% of comonomer.

Preferably the polypropylenes used in the present invention, irrespectively of whether used in the exterior or the interior component, are predominantly isotactic polypropylenes, meaning that they are characterized by high isotacticity, for which the content of mmmm pentads is a measure. The content of mmmm pentads is at least 95.0 % and most preferably at least 96.0 wt%. The isotacticity (mmmm %) is determined by NMR analysis according to the method described by G.J. Ray et al. in Macromolecules, vol. 10, n° 4, 1977, p. 773-778, on the dried product resulting from the extraction by boiling heptane of the xylene insoluble fraction.

The polypropylene of the exterior component preferably comprises at least 200 ppm of a primary antioxidant; more preferably it comprises at least 200 ppm of a primary antioxidant and at least 500 ppm of a secondary antioxidant.

The primary antioxidant is a chemical compound that is capable of interfering with the chain propagation step in the thermal oxidation of polymers. Said primary antioxidant is preferably chosen from the group consisting of sterically hindered phenols, lactones and blends thereof. Most preferably said primary antioxidant is chosen from the group of sterically hindered phenols and blends thereof. Sterically hindered phenols suited for use in the present invention are characterized in that they comprise a phenol group, which in both positions neighboring the hydroxyl group is substituted with bulky alkyl substituents, such as tert-butyl. Examples of suited sterically hindered phenols are Irganox 1010 (CAS nr. 6683-19-8), Irganox 1035 (CAS nr. 41484-35-9), Irganox 1076 (CAS nr 2082-79-3) , Irganox 1081 (CAS nr. 90-66-4), Irganox 1330 (CAS nr. 1709-70-2), Irganox 1425 (CAS nr. 65140-91-2), and Irganox 3114 (CAS nr. 27676-62-6). Of these Irganox 1010, Irganox 1076 and Irganox 1425 WL are more preferred. Most preferred are Irganox 1010 and Irganox 1076. An example of a suitable lactone is Irganox HP 136 (CAS nr. 181314-48-7).

The secondary antioxidant is a chemical compound capable of destroying hydroperoxide groups, which are responsible for chain-initiation and chain-branching in the decomposition of polymers, by the decomposition of hydroperoxides without intermediate formation of free radicals. Preferred secondary antioxidants are phosphites and blends thereof. Phosphites suited for use in the present invention are Irgafos 168 (CAS nr. 31570-04-4), Irgafos 38 (CAS nr. 145650-60-8), Irgafos P-EPQ (CAS nr. 119345-01-6) and Ultranox 626 (CAS nr. 26741-53-7). Irgafos 168 is the most preferred.

Irganox and Irgafos are tradenames of Ciba Specialty Chemicals, now being part of BASF AG.

If said primary antioxidant is present, more preferably it is comprised in the polypropylene of the exterior component in at least 250 ppm, even more preferably in at least 300 ppm, still even more preferably in at least 350 ppm, and most preferably in at least 400 ppm. If present said primary antioxidant is comprised in the polypropylene of the exterior component in at most 2000 ppm, and most preferably in at most 1000 ppm. All amounts given are relative to the total weight of the polypropylene of the exterior component.

If said secondary antioxidant is present, more preferably it is comprised in the polypropylene of the exterior component in at least 700 ppm, and most preferably in at least 900 ppm. If present, said secondary antioxidant is comprised in the polypropylene of the exterior component in at most 5000 ppm, more preferably in at most 4000 ppm, even more preferably in at most 3000 ppm, still even more preferably in at most 2000 ppm and most preferably in at most 1500 ppm. All amounts are given relative to the total weight of the polypropylene of the exterior component.

Without wishing to be bound by theory it is believed that the addition of the primary antioxidant or the primary and secondary antioxidants inhibits the degradation of the polypropylene to keep it below a threshold, the surpassing of which would contribute to a decrease in the mechanical properties of the fibers and the nonwovens comprising such fibers.

The polypropylenes used in the present invention either in the exterior or the interior component and the thermoplastic polymers used in the interior component may also contain further additives such as, by way of example, antioxidants other than the ones described above, light stabilizers, acid scavengers, lubricants, antistatic additives, and colorants. An overview of suitable additives as well as on the antioxidants described above is given for example in the Plastics Additives Handbook, 5th edition, ed. Hans Zweifel, Carl Hanser Verlag, 2001.

The bicomponent fibers as described above may be comprised in nonwovens, particularly in thermally bonded nonwovens or in spunbond nonwovens. It is preferred that such nonwovens comprise at least 50 wt%, preferably at least 70 wt% or 90 wt%, more preferably at least 95 wt% and most preferably that they consist of the bicomponent fibers of the present invention.

Surprisingly, the bicomponent fibers and nonwovens in accordance with the present invention are characterized by no or at most very little improvement in softness as had been expected from the use of the higher melt flow polypropylene as exterior component.

However, equally surprisingly it has been found that the nonwovens, especially the spunbond nonwovens, of the present invention show an increase of around 10 % in tenacity. It needs to be emphasized that the tenacity increase was observed in machine as well as in cross-machine direction when compared to nonwovens comprising fibers made from the polypropylene of the interior component only.

The present inventors have also been surprised that the increase in tenacity that was observed on the nonwovens, especially the spunbond nonwovens, of the present invention was not accompanied by a decrease in elongation but on the contrary by an increase in elongational properties. Thus, the present invention allows the production of nonwovens that at the same time have improved tenacity and elongation, and this in machine as well as cross-machine direction.

Nonwovens comprising the bicomponent fibers of the present invention may be used to form a composite of nonwoven layers or a laminate with film. A composite according to the present invention comprises a spunbond nonwoven layer (S) according to the present invention and/or a melt blown nonwoven layer (M). The composite can for example be of the SS, SSS, SMS, SMMSS or any other type. A laminate according to the present invention comprises a spunbond nonwoven layer (S) according to the present invention and a film layer (F) The laminate can be of the SF, SFS or any other type. Preferably, the film is a polyolefin film. The film of said laminate may be a breathable barrier film, thus resulting in a laminate with breathable properties.

The bicomponent fibers of the present invention as well as the nonwovens, composites and laminates comprising them are produced by methods well known to the person skilled in the art.

For the production of the bicomponent fibers of the present invention a polypropylene composition comprising the polypropylene as defined above for the exterior component is molten in a first extruder. Preferably, said polypropylene composition comprises at least 50 wt%, more preferably at least 70 wt% or 90 wt%, even more preferably at least 95 wt% or 97 wt% or 99 wt% of the polypropylene as defined above for the exterior component relative to the total weight of the exterior component; it is most preferred that the exterior layer consists of the polypropylene as defined above for the exterior component.

A thermoplastic polymer composition comprising a thermoplastic polymer as defined for the interior component is molten in a second extruder. Preferably said thermoplastic polymer composition comprises at least 50 wt%, more preferably at least 70 wt% or 90 wt%, even more preferably at least 95 wt% or 97 wt% or 99 wt% of said thermoplastic polymer as defined for the interior component relative to the total weight of the exterior component; it is most preferred that the interior layer consists of said thermoplastic polymer as defined for the interior component.

The molten thermoplastic polymer composition is then extruded from a number of fine, usually circular, capillaries of a spinneret. The molten polypropylene composition is extruded from a number of fine openings surrounding said capillaries. The extrudates from capillary and corresponding fine opening (Depending upon the type or bicomponent fiber to be produced it can also mean the extrudates from one or more capillaries and one or more surrounding fine opening that are intended to form a single filament.) are then combined to form a single, usually circular, filament of an intermediate diameter, whereby the extruded polypropylene composition forms the exterior component and the extruded thermoplastic polymer composition forms the interior component. In an optional step the intermediate diameter of the filaments is rapidly reduced to a final diameter (drawing step). In the drawing step the fibers can be drawn over heated rolls or in a heated oven to further reduce the intermediate diameter to a final diameter and increase the tenacity of the fibers. If no further drawing step is performed the intermediate diameter is the final diameter. The production of bicomponent fibers is for example described in F. Fourné, Synthetische Fasern, Carl Hanser Verlag, 1995, chapter 5.2 or in B.C. Goswami et al., Textile Yarns, John Wiley & Sons, 1977, p. 371-376.

The nonwovens comprising the bicomponent fibers of the present invention may be produced either by thermal bonding of the bicomponent fibers of the present invention or by the spunbonding process. Preferably, the nonwovens of the present invention are produced by the spunbonding process.

Stated in general terms, the nonwovens are produced by collecting the bicomponent fibers of the present invention on a support and subsequently bonding the collected fibers to form a bonded nonwoven.

For the production of thermally bonded nonwovens the bicomponent fibers of the present invention are cut into staple fibers having a length in the range from 5 to 30 mm. Said staple fibers are then carded, i.e. collected as a more or less continuous non-consolidated web on a support. In a final step the non-consolidated web is consolidated by thermal or chemical bonding, with thermal bonding being preferred.

For the spunbonding process fiber formation can be accomplished either by using one single spinneret with a large number of holes, generally several thousand, or by using several smaller spinnerets with a correspondingly smaller number of holes per spinneret. The combined extrudates with the polypropylene composition forming the exterior component and the thermoplastic polymer composition forming the interior component are quenched by a current of cold air. The diameter of the filaments is then rapidly reduced to a final diameter by a stream of high-pressure air. Air velocities in the drawdown step can be of several thousand meters per minute. After drawdown the filaments are collected on a support, for example a wire mesh belt, thus creating a first fabric, which may then be passed through compaction rolls and finally goes through a bonding step. Bonding of the fabric may be accomplished by thermobonding, hydroentanglement, needlepunching, or chemical bonding.

In comparison to the production of the well known bicomponent fibers having a polypropylene as interior component and a polyethylene as exterior component the fibers of the present invention proved very easy to process. No problems were encountered in the production of the nonwovens, especially the spunbond nonwovens, comprising the bicomponent fibers of the present invention.

In addition the bicomponent fibers and nonwovens of the present invention proved to also have the advantage of being more easily produced that fibers and nonwovens made from a commercial polypropylene of melt flow index 25 dg/min (measured according to ISO 1133, condition L, 230°C, 2.16 kg) and of narrow molecular weight distribution. Without wishing to be bound by theory it is believed that this is due to the higher melt flow index of the polypropylene used in the exterior component of the bicomponent fibers and nonwovens of the present invention. Interestingly, the higher melt flow index of the polypropylene in the exterior component does not lead to a loss in mechanical properties of the bicomponent nonwovens of the present invention when comprised of fibers having comparable titer but rather to an increase in both, tenacity and elongational properties in both directions, machine and cross-machine direction.

One or more nonwovens in accordance with the present invention may be applied to one or more other nonwovens, which may but need not be in accordance with the present invention, to form a composite as described above. Preferably the one or more other nonwovens are thermally bonded nonwovens, spunbond nonwovens or melt blown nonwovens. Spunbond nonwovens are most preferred.

One of more nonwovens in accordance with the present invention may be laminated to a film to form a laminate. The film preferably is a polyolefin film. The film may be a breathable barrier film, thus resulting in a laminate with breathable properties.

The fibers, nonwovens, composites and laminates of the present invention may be used in hygiene articles, such as baby diapers, adult incontinence products, female hygiene products, and wipes, or in products for the construction industry or for agriculture, or for medical drapes and gowns, protective garments, lab coats etc.

### Examples

### TEST METHODS

The melt flow index was measured according to norm ISO 1133, condition L, using a weight of 2.16 kg and a temperature of 230 °C.

Molecular weights are determined by Size Exclusion Chromatography (SEC) at high temperature (145°C). A 10 mg PP sample is dissolved at 160°C in 10 ml of TCB (technical grade) for 1 hour. The analytical conditions for the Alliance GPCV 2000 from WATERS are :
- Volume : +/- 400µl
- Injector temperature : 140°C
- Column and detector : 145°C
- Column set: 2 Shodex AT-806MS and 1 Styragel HT6E
- Flow rate 1 ml/min
- Detector: Refractive index
- Calibration : Narrow standards of polystyrene
- Calculation : Based on Mark-Houwink relation (log(M_{PP}) = log(M_{PS}) - 0.25323)

The isotacticity (mmmm %) is determined by NMR analysis according to the method described by G.J. Ray et al. in Macromolecules, vol. 10, n° 4, 1977, p. 773-778. It is performed on the dried product resulting of the extraction by boiling heptane of the xylene insoluble fraction.

The xylene insoluble fraction was obtained as follows: Between 4.5 and 5.5 g of propylene polymer were weighed into a flask and 300 ml xylene were added. The xylene was heated under stirring to reflux for 45 minutes. Stirring was continued for 15 minutes exactly without heating. The flask was then placed in a thermostated bath set to 25°C +/- 1 °C for 1 hour. The solution was filtered through Whatman n° 4 filter paper with the xylene insoluble fraction being retained on the filter.

The heptane insoluble fraction was isolated as follows: The xylene insoluble fraction (see above) was dried in air for a minimum of 3 days and manually ground into small pieces, of which ca. 2 g were weighed into the extraction thimble of a Soxleth extractor and extracted with heptane under reflux for 15 hours. The heptane insoluble fraction was recovered from the thimble, and dried in air for a minimum of 4 days.

Tensile strength and elongation of the nonwovens were measured according to ISO 9073-3:1989.

### POLYPROPYLENES

Nonwovens were produced using a polypropylene homopolymer, denoted as PP1, and a commercial polypropylene homopolymer, denoted as PP2. An overview of their properties is given in table 1.

**Table 1**

| | | PP1 | PP2 |
|---|---|---|---|
| Degradation ratio MFI₁/MFI₂ | | 0.2 | 0.08 |
| Final MFI | dg/min | 60 | 25 |
| Mₙ | kDa | 33 | 46 |
| M_{w} | kDa | 152 | 189 |
| M_{z} | kDa | 431 | 452 |
| MWD = M_{w}/Mₙ | | 4.6 | 4.1 |

Both, PP1 and PP2, contained 400 ppm of Irganox 3114 as primary antioxidant and 800 ppm of Irgafos 168 as secondary antioxidant.

### SPUNBOND NONWOVEN

Polypropylenes PP1 and PP2 were used to produce the following spunbond nonwovens
- Example 1: - Bicomponent nonwoven with PP1 as exterior component and PP2 as interior component wherein the exterior layer comprised 30 wt% of the total weight of the fibers
- Comparative example 1: - Nonwoven made from PP2

The spunbond nonwovens were produced on a 1.1 m wide Reicofil 4 line with a single beam having about 6800 holes per meter length, the holes having a diameter of 0.6 mm.. The nonwoven had a fabric weight of 12 g/m². The nonwoven were thermally bonded using an embossed roll. Further processing conditions are given in table 2. The bonding roll temperature reported in table 2 is the bonding temperature at which the highest values for elongation were obtained. Properties of the nonwoven obtained under these conditions are shown in table 3.

**Table 2**

| | | | Ex. 1 | Comp. ex. 1 |
|---|---|---|---|---|
| Belt speed | | m/min | 300 | 300 |
| Throughput | | Kg/h/m | 220 | 220 |

| Extruder temperature | | | | |
|---|---|---|---|---|
| | - Exterior component | °C | 240 | 250 |
| | - Interior component | °C | 250 | n.a. |

| Melt temperature at the die | | | | |
|---|---|---|---|---|
| | - Exterior component | °C | 247 | 256 |
| | - Interior component | °C | 249 | 249 |
| Cabin pressure | | Pa | 8000 | 8000 |
| Nip pressure | | N/mm | 80 | 80 |
| Calender temperature (set point) for max. elongation | | °C | 152 | 155 |

**Table 3**

| | | Ex. 1 | Comp. ex. 1 |
|---|---|---|---|
| Filament titer | den | 1.25 | 1.16 |
| Tensile strength @ max MD | N/5cm | 34.0 | 31.5 |
| Tensile strength @ max CD | N/5cm | 18.0 | 17.1 |
| Elongation MD | % | 81 | 68 |
| Elongation CD | % | 72 | 71 |

The results clearly demonstrate the advantages of the present invention:
- Because the polypropylene of the exterior component has a higher melt flow index than the current commercial polypropylene spunbond grades (as exemplified by PP2) the extruder temperature of the respective extruder could be lowered. This leads to a reduction in energy consumption but also to less thermal degradation of the polypropylene.
- The combination of polypropylene PP1 of higher melt flow index as exterior component and polypropylene PP2 of lower melt flow index as interior component allowed to improve the strength of the nonwoven in machine direction as well as in cross-machine direction.
- At the same time as the nonwoven strength could be increased the bicomponent nonwovens of the present invention allowed increasing the elongational properties, which is quite surprising as the elongation normally decreases when strength increases and vice versa.

Thus, the results show that the fibers and nonwovens in accordance with the present invention have improved properties in comparison to the fibers and nonwovens of the prior art. The present invention further allows the production of bicomponent fibers and nonwovens based on polypropylene only, without having to revert to the use of polyethylene in the exterior component, thus facilitating the production of such bicomponent fibers and nonwovens.

## Claims

1. Bicomponent fiber comprising
(a) an exterior component covering at least 50 % of the surface of the bicomponent fiber, and
(b) an interior component comprising a thermoplastic polymer,
wherein the exterior component comprises a polypropylene, which has been degraded chemically or thermally from a first melt flow index MFI₁ (measured according to ISO 1133, condition L, 230°C, 2.16 kg) to a second melt flow index MFI₂ (measured according to ISO 1133, condition L, 230°C, 2.16 kg), such that the second melt flow index MFI₂ is in the range from 50 dg/min to 300 dg/min and such that the degradation ratio MFI₁/MFI₂ is at least 0.10 and at most 0.80.

2. Bicomponent fiber according to claim 1, wherein the exterior component comprises said polypropylene in at least 50 wt% relative to the total weight of the exterior component.

3. Bicomponent fiber according to claim 1 or claim 2, wherein the exterior component comprises a polypropylene, said polypropylene comprising at least 200 ppm, relative to the weight of said polypropylene, of a primary antioxidant.

4. Bicomponent fiber according to claim 3, wherein the exterior component comprises a polypropylene, said polypropylene comprising at least 200 ppm, relative to the total weight of said polypropylene, of a primary antioxidant and at least 500 ppm, relative to the total weight of said polypropylene, of a secondary antioxidant.

5. Bicomponent fiber according to claims 1 to 4, wherein the thermoplastic polymer of the interior component is a polypropylene different from the polypropylene of the exterior component.

6. Nonwoven comprising the bicomponent fiber of any of claims 1 to 5.

7. Composite and laminate comprising the nonwoven of claim 6.

8. Process for the production of bicomponent fibers comprising the steps of
(a) polymerizing propylene and one or more optional comonomers with a polymerization catalyst to produce a polypropylene having a first melt flow index MFI₁ (measured according to ISO 1133, condition L, 230°C, 2.16 kg),
(b) thermally or chemically degrading the polypropylene obtained in step (a) to a second melt flow index MFI₂ (measured according to ISO 1133, condition L, 230 °C, 2.16 kg),
(c) melting a polypropylene composition comprising the polypropylene obtained in step (b) in a first extruder to form a molten polypropylene composition,
(d) melting a thermoplastic polymer composition comprising a thermoplastic polymer in a second extruder to form a molten thermoplastic polymer composition,
(e) extruding the molten thermoplastic polymer composition from a number of fine, usually circular, capillaries of a spinneret,
(f) extruding the molten polypropylene composition of step (c) from a number of fine openings surrounding said capillaries of step (e), and
(g) combining the extrudates of steps (e) and (f) to form a single filament of an intermediate diameter, such that the extrudates of step (f) form an exterior component covering at least 50 % of the surface of the so-produced filament,
wherein the polypropylene obtained in step (b) has a second melt flow index MFI₂ (measured according to ISO 1133, condition L, 230°C, 2.16 kg) in the range from 50 dg/min to 300 dg/min and wherein the degradation ratio MFI₁/MFI₂ is at least 0.10 and at most 0.80.

9. Process according to claim 8, wherein the polypropylene in step (a) is produced by a Ziegler-Natta polymerization catalyst.

10. Process according to claim 8 or claim 9, wherein the exterior component and the interior component are further defined according to claims 2 to 5.

11. Process according to any of claims 8 to 10, wherein the process further comprises the step of
(h) rapidly reducing the intermediate diameter of the filaments extruded in the previous step to a final diameter.

12. Process according to any of claims 8 to 10, wherein the process further comprises the step of
(i) collecting the filaments obtained in step (g) or (h) on a support, and
(k) subsequently bonding the collected filaments to form a bonded nonwoven.

13. Process according to any of claims 8 to 12, further comprising the step of
(I-1) laminating a film to the bonded nonwoven obtained in step (k) to form a laminate

14. Process according to any of claims 8 to 12, further comprising the step of
(I-2) applying a spunbond and/or a meltblown nonwoven to the bonded nonwoven obtained in step (k).

15. Process according to any of claims 8 to 14, wherein the bonded nonwoven is a spunbond nonwoven.

## Patentansprüche

1. Zweikomponentenfaser, umfassend:
(a) eine äußere Komponente, die mindestens 50 % der Oberfläche der Zweikomponentenfaser bedeckt, und
(b) eine innere Komponente, die ein thermoplastisches Polymer umfasst, wobei die äußere Komponente ein Polypropylen umfasst, das chemisch oder thermisch von einem ersten Schmelzindex MFI₁ (gemessen nach ISO 1133, Bedingung L, 230 °C, 2,16 kg) auf einen zweiten Schmelzindex MFI₂ (gemessen nach ISO 1133, Bedingung L, 230 °C, 2,16 kg) degradiert wurde, derart dass der zweite Schmelzindex MFI₂ im Bereich von 50 dg/min bis 300 dg/min liegt und derart dass das MFI₁/MFI₂-Degradationsverhältnis mindestens 0,10 und höchstens 0,80 beträgt.

2. Zweikomponentenfaser nach Anspruch 1, wobei die äußere Komponente das Polypropylen in mindestens 50 Gew.-% bezogen auf das Gesamtgewicht der äußeren Komponente umfasst.

3. Zweikomponentenfaser nach Anspruch 1 oder 2, wobei die äußere Komponente ein Polypropylen umfasst, wobei das Polypropylen mindestens 200 ppm eines primären Antioxidationsmittels bezogen auf das Gewicht des Polypropylens umfasst.

4. Zweikomponentenfaser nach Anspruch 3, wobei die äußere Komponente ein Polypropylen umfasst, wobei das Polypropylen mindestens 200 ppm eines primären Antioxidationsmittels bezogen auf das Gesamtgewicht des Polypropylens und mindestens 500 ppm eines sekundären Antioxidationsmittels bezogen auf das Gesamtgewicht des Polypropylens umfasst.

5. Zweikomponentenfaser nach Anspruch 1 bis 4, wobei das thermoplastische Polymer der inneren Komponente ein vom Polypropylen der äußeren Komponente verschiedenes Polypropylen ist.

6. Vlies, umfassend die Zweikomponentenfaser nach einem der Ansprüche 1 bis 5.

7. Verbundstoff und Laminat, umfassend das Vlies nach Anspruch 6.

8. Verfahren zur Herstellung von Zweikomponentenfasern, umfassend die folgenden Schritte:
(a) Polymerisieren von Propylen und einem oder mehreren optionalen Comonomeren mit einem Polymerisationskatalysator, um ein Polypropylen mit einem ersten Schmelzindex MFI₁ (gemessen nach ISO 1133, Bedingung L, 230 °C, 2,16 kg) zu erzeugen,
(b) thermisches oder chemisches Degradieren des in Schritt (a) erhaltenen Polypropylens auf einen zweiten Schmelzindex MFI₂ (gemessen nach ISO 1133, Bedingung L, 230°C, 2,16 kg),
(c) Schmelzen einer Polypropylenzusammensetzung, die das in Schritt (b) erhaltene Polypropylen umfasst, in einem ersten Extruder, um eine geschmolzene Polypropylenzusammensetzung zu bilden,
(d) Schmelzen einer thermoplastischen Polymerzusammensetzung, die ein thermoplastisches Polymer umfasst, in einem zweiten Extruder, um eine geschmolzene thermoplastische Polymerzusammensetzung zu bilden,
(e) Extrudieren der geschmolzenen thermoplastischen Polymerzusammensetzung aus einer Anzahl von feinen, üblicherweise kreisförmigen, Kapillaren einer Spinndüse,
(f) Extrudieren der geschmolzenen Polypropylenzusammensetzung von Schritt (c) aus einer Anzahl von feinen Öffnungen, welche die Kapillare von Schritt (e) umgeben, und
(g) Kombinieren der Extrudate von Schritt (e) und (f), um ein einziges Filament eines Zwischendurchmessers zu bilden, derart dass die Extrudate von Schritt (f) eine äußere Komponente bilden, die mindestens 50 % der Oberfläche des auf diese Weise hergestellten Filaments bedeckt,
wobei das in Schritt (b) erhaltene Polypropylen einen zweiten Schmelzindex MFI₂ (gemessen nach ISO 1133, Bedingung L, 230 °C, 2,16 kg) im Bereich von 50 dg/min bis 300 dg/min aufweist, und wobei das MFI₁/MFI₂-Degradationsverhältnis mindestens 0,10 und höchstens 0,80 beträgt.

9. Verfahren nach Anspruch 8, wobei das Polypropylen in Schritt (a) durch einen Ziegler-Natta-Polymerisationskatalysator erzeugt wird.

10. Verfahren nach Anspruch 8 oder 9, wobei die äußere Komponente und die innere Komponente ferner nach Anspruch 2 bis 5 definiert sind.

11. Verfahren nach einem der Ansprüche 8 bis 10, wobei das Verfahren ferner den folgenden Schritt umfasst:
(h) schnelles Verringern des Zwischendurchmessers der im vorherigen Schritt extrudierten Filamente auf einen Enddurchmesser.

12. Verfahren nach einem der Ansprüche 8 bis 10, wobei das Verfahren ferner die folgenden Schritte umfasst:
(i) Sammeln der in Schritt (g) oder (h) erhaltenen Filamente auf einem Träger, und
(k) anschließendes Binden der gesammelten Filamente, um ein gebundenes Vlies zu bilden.

13. Verfahren nach einem der Ansprüche 8 bis 12, ferner umfassend den Schritt (I-1) des Laminierens eines Films auf das in Schritt (k) erhaltene gebundene Vlies, um ein Laminat zu bilden.

14. Verfahren nach einem der Ansprüche 8 bis 12, ferner umfassend den Schritt (1-2) des Aufbringens eines spinngebundenen und/oder schmelzgeblasenen Vlieses auf das in Schritt (k) erhaltene gebundene Vlies.

15. Verfahren nach einem der Ansprüche 8 bis 14, wobei das gebundene Vlies ein spinngebundenes Vlies ist.

## Revendications

1. Fibre bicomposant comprenant
(a) un composant extérieur couvrant au moins 50 % de la surface de la fibre bicomposant, et
(b) un composant intérieur comprenant un polymère thermoplastique,
dans laquelle le composant extérieur comprend un polypropylène, qui a été dégradé chimiquement ou thermiquement d'un premier indice de fluage MFI₁ (mesuré conformément à la norme ISO 1133, condition L, 230 °C, 2,16 kg) à un deuxième indice de fluage MFI₂ (mesuré conformément à la norme ISO 1133, condition L, 230 °C, 2,16 kg), de manière à ce que le deuxième indice de fluage MFI₂ soit dans la plage de 50 dg/min à 300 dg/min et de manière à ce que le rapport de dégradation MFI₁/MFI₂ soit d'au moins 0,10 et d'au plus 0,80.

2. Fibre bicomposant selon la revendication 1, dans laquelle le composant extérieur comprend ledit polypropylène en une concentration d'au moins 50 % en poids par rapport au poids total du composant extérieur.

3. Fibre bicomposant selon la revendication 1 ou la revendication 2, dans laquelle le composant extérieur comprend un polypropylène, ledit polypropylène comprenant au moins 200 ppm, par rapport au poids dudit polypropylène, d'un antioxydant primaire.

4. Fibre bicomposant selon la revendication 3, dans laquelle le composant extérieur comprend un polypropylène, ledit polypropylène comprenant au moins 200 ppm, par rapport au poids total dudit polypropylène, d'un antioxydant primaire et au moins 500 ppm, par rapport au poids total dudit polypropylène, d'un antioxydant secondaire.

5. Fibre bicomposant selon les revendications 1 à 4, dans laquelle le polymère thermoplastique du composant intérieur est un polypropylène différent du polypropylène du composant extérieur.

6. Non-tissé comprenant la fibre bicomposant selon l'une quelconque des revendications 1 à 5.

7. Composite et stratifié comprenant le non-tissé selon la revendication 6.

8. Procédé de production de fibres bicomposants comprenant les étapes consistant à
(a) polymériser du propylène et un ou plusieurs comonomères optionnels avec un catalyseur de polymérisation pour produire un polypropylène ayant un premier indice de fluage MFI₁ (mesuré conformément à la norme ISO 1133, condition L, 230 °C, 2,16 kg),
(b) dégrader thermiquement ou chimiquement le polypropylène obtenu lors de l'étape (a) à un deuxième indice de fluage MFI₂ (mesuré conformément à la norme ISO 1133, condition L, 230 °C, 2,16 kg),
(c) faire fondre une composition de polypropylène comprenant le polypropylène obtenu lors de l'étape (b) dans une première extrudeuse pour former une composition de polypropylène fondue,
(d) faire fondre une composition de polymère thermoplastique comprenant un polymère thermoplastique dans une deuxième extrudeuse pour former une composition de polymère thermoplastique fondue,
(e) extruder la composition de polymère thermoplastique fondue à partir d'un certain nombre de capillaires fins, généralement circulaires, d'une filière,
(f) extruder la composition de polypropylène fondue de l'étape (c) à partir d'un certain nombre d'ouvertures fines entourant lesdits capillaires de l'étape (e), et
(g) combiner les extrudats des étapes (e) et (f) pour former un filament unique de diamètre intermédiaire, de manière à ce que les extrudats de l'étape (f) forment un composant extérieur couvrant au moins 50 % de la surface du filament ainsi produit,
dans lequel le polypropylène obtenu lors de l'étape (b) a un deuxième indice de fluage MFI₂ (mesuré conformément à la norme ISO 1133, condition L, 230 °C, 2,16 kg) dans la plage de 50 dg/min à 300 dg/min et dans lequel le rapport de dégradation MFI₁/MFI₂ est d'au moins 0,10 et d'au plus 0,80.

9. Procédé selon la revendication 8, dans lequel le polypropylène de l'étape (a) est produit par un catalyseur de polymérisation de type Ziegler-Natta.

10. Procédé selon la revendication 8 ou la revendication 9, dans lequel le composant extérieur et le composant intérieur sont en outre définis selon les revendications 2 à 5.

11. Procédé selon l'une quelconque des revendications 8 à 10, dans lequel le procédé comprend en outre l'étape consistant à
(h) réduire rapidement le diamètre intermédiaire des filaments extrudés lors de l'étape précédente à un diamètre final.

12. Procédé selon l'une quelconque des revendications 8 à 10, dans lequel le procédé comprend en outre l'étape consistant à
(i) récupérer les filaments obtenus lors de l'étape (g) ou (h) sur un support, et
(k) ensuite lier les filaments récupérés pour former un non-tissé lié.

13. Procédé selon l'une quelconque des revendications 8 à 12, comprenant en outre l'étape consistant à
(I-1) laminer un film sur le non-tissé lié obtenu lors de l'étape (k) pour former un stratifié.

14. Procédé selon l'une quelconque des revendications 8 à 12, comprenant en outre l'étape consistant à
(I-2) appliquer un filé-lié et/ou un non-tissé produit par fusion-soufflage sur le non-tissé lié obtenu lors de l'étape (k).

15. Procédé selon l'une quelconque des revendications 8 à 14, dans lequel le non-tissé lié est un non-tissé filé-lié.
